

Patented Mar. 27, 1928.

1,664,323

# UNITED STATES PATENT OFFICE.

TULLIO SARRA, OF SAN BRUNO, CALIFORNIA.

## PROCESS OF MAKING GUT STRINGS.

No Drawing.

Application filed March 22, 1926. Serial No. 96,668.

This invention relates to the manufacture of gut strings, such for example, as those used in tennis rackets, and the primary object of the invention is to provide a new and improved process of manufacturing gut strings from intestines which have been heretofore considered useless for this purpose, and to provide an improved and stronger string at cheaper cost.

10 Gut strings have heretofore been made principally from the intestines of such animals as lambs, sheep, hogs etc., the intestines of larger animals such as beef cattle not being suitable. As a result, the intestines of the smaller animals have been in such great demand for making gut strings that the cost of such strings is considerable, while the intestines of the larger animals have remained a cheap by-product. It is an object of my invention to provide a new process whereby a better gut string can be made from these cheap intestines. Obviously, this new process adapts a cheap raw material, otherwise useless for this purpose, 25 to this new use.

I have found that while bovine intestines as a whole are not suited to the manufacture of gut strings, the inner layer thereof is quite suited to this purpose. It is another object of my invention to provide a process for separating this inner layer from the remaining portion of the intestines, whereby the same can be used for the purpose stated.

In the following specification, I have specifically described my improved process and have therein defined specific proportions and materials which I may use. It will be understood however, that the details stated may be varied within reasonable limits, and that the materials and proportions mentioned are considered as also including the equivalents thereof. Also, while I have defined my invention as being particularly applicable to use on bovine intestines, the same may of course be likewise applicable to the intestines of other like animals.

In carrying out my invention, I may proceed as follows.

The intestines after being thoroughly washed, are soaked in a 5% potassium hydroxide solution until the outer layer is loosened. They are then slit lengthwise into two ribbons, and the outer layer thereof peeled off.

55 The remaining inner layers are then again soaked in a stronger potassium hydroxide

solution of 7½% strength, until the remaining outer layer is loosened from the inner layer. This outer layer is then peeled from the inner layer.

60 The remaining inner layer is then soaked in a stronger potassium hydroxide solution of 10% strength for the purpose of softening the gut and the fat thereon. After this soaking, the gut is run through a machine 65 having a series of rapidly revolving knives, which clean the fat therefrom.

The processing of the intestines is now complete and the remaining inner layer is ready to be manufactured into strings. I 70 preferably proceed as follows.

I soak this gut in a 12½% potassium hydroxide solution for five days, the solution being changed each day. This soaking strengthens the gut so that it can be twisted 75 into strings.

Gut strings are ordinarily made from several plies of gut laid together and twisted into a single string. The number of plies used depends upon the size of string to be 80 made and upon the width of the gut. In manufacturing the strings, I ordinarily place from eight to fifteen of the gut ribbons together and twist the same into a string. This twisting and finishing operation is the same as that now used in manufacturing gut strings and further description thereof herein is therefore believed to be unnecessary.

Having thus described my invention, what 90 I claim is:

1. The process of making gut strings from the inner layer of bovine intestines which comprises separating the outer layers from the inner layer of such intestines by soaking 95 the same in a solution of a hydroxide of an alkali metal which loosens the layers and then removing the outer layer and thereafter treating the inner layer with a similar solution to strengthen the same and twisting 100 the resulting product into gut strings.

2. The process of making gut strings which comprises soaking bovine intestines in a caustic alkali solution, separating the outer layers thereof from the inner layer, soaking 105 the inner layer in a similar solution to soften the gut and the fat thereon, removing the fat therefrom, soaking the gut in a similar solution to strengthen the gut, and thereafter placing a plurality of layers of the 110 gut together and twisting the same to form a string.

3. The process of making gut strings which comprises soaking bovine intestines in a potassium hydroxide solution, separating the outer layers thereof from the 5 inner layer, soaking the inner layer in a potassium hydroxide solution to soften the gut and the fat thereon, removing the fat therefrom, soaking the gut in a stronger potassium hydroxide solution to strengthen 10 the gut, and thereafter placing a plurality of layers of the gut together and twisting the same to form a string.

4. The process of making gut strings which comprises soaking bovine intestines in a potassium hydroxide solution, separating the outer layer therefrom, again soaking the remaining gut in a stronger potassium hydroxide solution, separating the remaining outer layer therefrom, again soaking 15 the remaining gut in a stronger potassium hydroxide solution to soften the gut and the fat thereon, removing the fat, thereafter soaking the gut in a substantially 12½% potassium hydroxide solution to strengthen the gut, and thereafter placing a plurality of layers of the gut together and twisting the same to form a string.

tassium hydroxide solution to strengthen the gut, and thereafter placing a plurality of 25 layers of the gut together and twisting the same to form a string.

5. The process of making gut strings which comprises soaking bovine intestines in a substantially 5% potassium hydroxide solution, slitting the same lengthwise into two ribbons and separating the outer layer therefrom, again soaking the remaining gut in a substantially 7½% potassium hydroxide solution, separating the remaining outer 30 layer therefrom, again soaking the remaining gut in a substantially 10% potassium hydroxide solution to soften the gut and the fat thereon, removing the fat, thereafter 35 soaking the gut in a substantially 12½% potassium hydroxide solution to strengthen the gut, and thereafter placing a plurality of layers of the gut together and twisting the same to form a string.

In testimony whereof I affix my signature.

TULLIO SARRA.